

[54] **METHOD OF PREPARATION OF SINGLE CRYSTAL FILMS**

[75] Inventors: **Bernard Ferrand; Francis Forrat; Yves Grange, all of Grenoble; Jean-Claude Joubert, Venon; Jean Mareschal, Gieres, all of France**

[73] Assignee: **Commissariat a l'Energie Atomique, Paris, France**

[22] Filed: **May 22, 1972**

[21] Appl. No.: **255,549**

[30] **Foreign Application Priority Data**

May 25, 1971 France ..... 71.18889

[52] U.S. Cl. .... **117/235, 117/113, 423/263, 423/594**

[51] Int. Cl. .... **H01f 10/02**

[58] **Field of Search** ..... 117/235-240, 117/113, 65.2; 423/594, 263

[56] **References Cited**

UNITED STATES PATENTS

3,047,429 7/1962 Stoller et al. ..... 117/235

|           |         |                                |
|-----------|---------|--------------------------------|
| 3,100,158 | 8/1963  | Lemaire et al. .... 117/235 X  |
| 3,404,026 | 10/1968 | Skudera et al. .... 117/235 UX |
| 3,429,740 | 2/1969  | Mee ..... 117/235 X            |
| 3,486,937 | 12/1969 | Linares ..... 117/235 X        |
| 3,573,099 | 3/1971  | Moore et al. .... 117/235 X    |
| 3,607,390 | 9/1971  | Comstock ..... 117/235 X       |
| 3,697,320 | 10/1972 | Hiskes ..... 117/235 X         |

*Primary Examiner*—William D. Martin

*Assistant Examiner*—Bernard D. Pianalto

*Attorney, Agent, or Firm*—Cameron, Kerkam, Sutton, Stowell & Stowell

[57] **ABSTRACT**

A method of preparation of a single-crystal thin film of a rare earth mixed oxide having a garnet structure of the formula  $T_3M_5O_{12}$  where M represents iron and T represents Yttrium. A single-crystal substrate is placed in an aqueous solution which is capable of liberating the constituents of the single-crystal film in situ; the solution is brought to a high temperature in order to dissolve the constituents of the single-crystal film; and these constituents are then deposited on the single-crystal substrate by recrystallization.

**10 Claims, No Drawings**

## METHOD OF PREPARATION OF SINGLE CRYSTAL FILMS

This invention relates to a method of preparation of single-crystal films, especially thin films of mixed oxides having a garnet structure.

The invention applies more particularly to the preparation of films of rare-earth single-crystals, synthetic double oxides corresponding to the formula  $T_3M_5O_{12}$  in which O is oxygen, M is iron which may be replaced either wholly or in part by aluminum, gallium or one of the transition elements having an atomic number within the range of 21 to 28 inclusive and in which T represents yttrium or one of the rare-earth elements having an atomic number within the range of 62 to 71, or alternatively a mixture of said rare-earth elements with each other or with yttrium.

The single-crystal films defined in the foregoing exhibit advantageous magnetic properties which permit their use in particular in the ultra-high frequency range (as resonant insulators, transducers, surface-wave amplifiers). These films can also be employed in logic and storage devices of the domain-displacement type.

One of the methods employed up to the present time for obtaining films of rare-earth single-crystals consists in growing a single crystal  $T_3M_5O_{12}$  on a seed of  $T_3M_5O_{12}$  by hydrothermal synthesis. This method was carried out in practice as follows: the  $T_3M_5O_{12}$  was dissolved in the polycrystalline form in a 20 M sodium hydroxide solution, in the bottom portion of an autoclave which was heated to 400°C; the single crystal was then recrystallized on a seed of  $T_3M_5O_{12}$  in the top portion of the autoclave which was heated to 375°C.

Another conventional method of formation of a single-crystal film consisted in growing a single crystal of  $T_3M_5O_{12}$  on a seed of GdGaG (gadolinium-gallium-garnet). A solution of 20 M NaOH or 20 M KOH at a temperature in the vicinity of 400°C was employed as solvent. But it proved difficult to apply this method to the preparation of thin films since the seed was frequently attacked by the solvent. There was also employed as solvent a 10 percent solution of  $NH_4Cl$  at temperatures in the vicinity of 550°C. However, the dissolution of the polycrystal  $T_3M_5O_{12}$  in the ammonium chloride was a very slow process, the seed of GdGaG was attacked by  $NH_4Cl$  and the single-crystal deposit was not uniform.

The method according to the invention overcomes the disadvantages recalled in the foregoing, especially insofar as it permits rapid dissolution of the constituents of the single crystal and consequently results in thin and homogeneous single-crystal films. One of the advantages of the invention lies in the fact that a single-crystal film can be deposited on a single-crystal substrate having a different chemical composition.

The method under consideration is primarily distinguished by the fact that a single-crystal substrate is placed in an aqueous solution which contains compounds having a base of constituents destined to form the single-crystal film and which is capable of liberating said constituents in situ, said solution is brought to a high temperature so as to dissolve said constituents, and said constituents are then deposited by recrystallization on said single-crystal substrate.

In a preferred mode of execution of the invention, thin single-crystal films of a rare-earth mixed oxide having a garnet structure, and corresponding to the for-

mula  $T_3M_5O_{12}$  as hereinabove defined, are deposited on a single-crystal substrate consisting of gadolinium-gallium-garnet-(GdGaG).

It will be readily understood that this composition is not intended to imply any limitation of the invention and the method can be employed for any other deposition of a single-crystal film of mixed oxides having a garnet structure on a predetermined single-crystal substrate. The method can also be applied to the preparation of single-crystal thin films of different magnetic compounds of garnets such as, for example, the orthoferrites of rare earths or the spinel ferrites.

The method according to the invention is carried out in an autoclave of heat-resisting steel lined with platinum, gold or silver. This autoclave is hermetically sealed by means of a system of gaskets of the "Bridgeman" type and connected to a manometer by a high-pressure flexible capillary wire. The autoclave is placed in a furnace having two separate heating zones which are regulated independently in order that it may thus be possible to control the temperature difference between the top and the bottom of the autoclave.

The method is carried into effect as follows:

The constituents which are intended to yield in situ the mixed oxide having a garnet structure by double decomposition are placed in an aqueous solution in the bottom of the autoclave which is the hot portion,

The single-crystal substrate is placed in the top of the autoclave which is the cold portion,

The aqueous solution is brought to a high temperature and high pressure in such manner as to decompose and dissolve the constituents of the mixed oxide, then to transport them into the cold portion of the autoclave in which they crystallize on the single-crystal substrate.

The temperature difference existing within the autoclave gives rise to convection currents which facilitate the transport of material from the hot portion to the cold portion.

In accordance with one advantageous feature of the method forming the subject of this invention, the aqueous solution is constituted by a solution of a mixed salt of a metal and of an alkali metal and a hydroxide or a salt of rare earth or of yttrium. For example, it is possible to employ  $NaFeO_2$  or  $KFeO_2$  and  $Y(OH)_3$ . Double decomposition results in formation on the one hand of sodium hydroxide or of potassium having a low concentration which acts as transporting and mineralizing agent and on the other hand of single-crystal film constituents which will be deposited on the single-crystal substrate.

In accordance with another feature of the method which forms the subject of the invention, the aqueous solution is constituted by a solution of a mixed salt of rare earth or of yttrium and of an alkali metal and a hydroxide or a salt of a metal.

For example, it is possible to carry out a double decomposition reaction between  $NaFeO_2$  and an yttrium salt such as, for example,  $YCl_2 \cdot 6H_2O$ ;  $Y(NO_3)_3$ . The salts which are formed, namely  $NaCl$ ,  $NaNO_3$ , accordingly act as transporting and mineralizing agents. It is also possible to carry out a double decomposition reaction between  $YNaO_2$  or  $YKO_2$  and newly precipitated  $Fe(OH)_3$  or a ferric salt such as, for example,  $FeCl_3$ ,  $Fe(NO_3)_3$ ,  $Fe_2(SO_4)_3$ .

In the method according to the invention, the operational temperature is within the range of 450°C to 550°C. A temperature difference of 20°C to 70°C is maintained between the bottom portion and the top portion of the autoclave.

The coefficient of filling in the autoclave is 0.4 to 0.6.

One example of application of the method according to the invention is given hereinafter without any implied limitation.

### EXAMPLE

Use is made of an autoclave having a useful volume of 130 cm<sup>3</sup> and lined with silver.

There are placed at the bottom of said autoclave 6 g of NaFeO<sub>2</sub>, 2.5 g of Y(OH)<sub>3</sub> and a sodium hydroxide solution consisting of 2.6 g of caustic soda in 60 cm<sup>3</sup> of water.

There is then fitted in position a platinum frame provided with a central screen having an opening of 20 percent.

At the top of said frame, there is placed a seed of Gd<sub>3</sub> Ga<sub>5</sub> O<sub>12</sub> which is cut at right angles to the direction (1, 1, 0).

The autoclave is closed and placed in a furnace having two temperature zones in order that the bottom portion of the autoclave should be at a temperature of 500°C and that the top portion should be at a temperature of 450°C.

The pressure is then 600 bars. The seeding process is carried out for a period of 24 hours.

At the end of this period, the autoclave is cooled rapidly and there is thus obtained a thin single-crystal film of Y<sub>3</sub>Fe<sub>5</sub>O<sub>12</sub> having a thickness of 2.5  $\mu$ .

What we claim is:

1. A method of preparation of a single-crystal thin film of a rare earth mixed oxide having a garnet structure of the formula T<sub>3</sub>M<sub>5</sub>O<sub>12</sub> where M represents iron and T represents yttrium, the steps of placing a single-

crystal substrate in an aqueous solution in an autoclave which contains compounds having a base of constituents to form the single-crystal film by liberating said constituents in situ by double decomposition, bringing said solution to a high temperature and high pressure to dissolve said constituents and then depositing said constituents by recrystallization on said single-crystal substrate, a temperature difference within the range of 20°C to 70°C being maintained between dissolution and deposition of the constituents.

2. A method according to claim 1, the coefficient of filling of the autoclave being between 0.4 to 0.6.

3. A method according to claim 1, the iron being at least partially replaced by a substance selected from the group consisting of aluminum, gallium and the transition elements having an atomic number within the range of 21 to 28 inclusive.

4. A method according to claim 1, T being a substance selected from the group consisting of the rare earth elements having an atomic number within the range of 62 to 71.

5. A method according to claim 1, the single-crystal substrate having a chemical composition different from that of the single-crystal film.

6. A method according to claim 1, the single-crystal substrate being gadolinium-gallium-garnet.

7. A method according to claim 1, the aqueous solution being a solution of a mixed salt of a metal and of an alkali metal and a hydroxide or a salt of rare earth or of yttrium.

8. A method according to claim 1, the aqueous solution being a solution of a mixed salt of rare earth or of yttrium and of an alkali metal and a hydroxide or a salt of a metal.

9. A method according to claim 8, wherein the solution contains NaFeO<sub>2</sub> and YCl<sub>2</sub>, 6H<sub>2</sub>O.

10. A method according to claim 1, the high temperature being between 400°C. and 550°C.

\* \* \* \* \*